

# United States Patent [19]

Corboy et al.

[11] 3,885,061

[45] May 20, 1975

[54] DUAL GROWTH RATE METHOD OF DEPOSITING EPITAXIAL CRYSTALLINE LAYERS

3,663,319 5/1972 Rose ..... 148/175  
3,669,769 6/1972 Badami et al. .... 117/106 A X  
3,765,960 10/1973 Boss et al. .... 117/106 A X

[75] Inventors: **John Francis Corboy**, Ringoes; **Glenn Wherry Cullen**, Princeton; **Nicholas Pastal**, Trenton, all of N.J.

[73] Assignee: **RCA Corp.**, Princeton, N.J.

[22] Filed: **Aug. 17, 1973**

[21] Appl. No.: **389,192**

[52] U.S. Cl. .... **117/201**; **117/106 A**; **148/175**

[51] Int. Cl. .... **C23c 11/00**

[58] Field of Search .... **117/106 A**, **201**; **148/175**

## [56] References Cited

### UNITED STATES PATENTS

3,189,494 6/1965 **Short** ..... 148/175

## OTHER PUBLICATIONS

Dumin et al., "Autodoping of Silicon Films Grown Epitaxially on Sapphire," Journal of the Electrochemical Society, May 1966, pp. 469-472.

Primary Examiner—Leon D. Rosdol

Assistant Examiner—Harris A. Pitlick

Attorney, Agent, or Firm—Glenn H. Bruestle; William S. Hill

## [57] ABSTRACT

Method of forming an epitaxial crystalline layer on a crystalline substrate by depositing a first portion at a rapid growth rate and a second portion at a slower growth rate.

5 Claims, 2 Drawing Figures



PATENTED MAY 20 1975

3,885,061

SHEET 1 OF 2



Fig. 1.



## DUAL GROWTH RATE METHOD OF DEPOSITING EPITAXIAL CRYSTALLINE LAYERS

The invention herein described was made in the course of or under contract No. F33615-C-1695 with the Department of the Air Force.

### BACKGROUND OF THE INVENTION

Device interaction in integrated circuits can be avoided by utilizing a type of circuit in which each active device occupies a separate island of single crystal semiconductor material deposited on an appropriate insulating substrate. For single crystal silicon films, for example, single crystal sapphire or spinel (magnesium aluminate) has proved to be a satisfactory substrate material. Hence this type of circuit has been referred to as an SOS (silicon-on-sapphire or silicon-on-spinel) circuit.

Experience has shown that it is difficult to make transistors in SOS work pieces which have all electrical characteristics as good as those of transistors made in bulk silicon work pieces. It has also been found that transistors in SOS work pieces vary widely in characteristics as growth parameters of the silicon films in which they are formed, are varied. This latter is due to the fact that properties of the grown silicon film, such as degree of crystalline perfection, vary with growth parameters such as growth rate of the film.

It has been found that, in the case of homoepitaxial growth, low growth rates tend to yield better crystalline quality than do high growth rates. Thus it would appear that heteroepitaxial films of silicon should also be deposited at relatively low growth rates in order to obtain optimum characteristics.

However, factors other than crystalline perfection must be considered. Heteroepitaxial silicon films are usually grown by passing a mixture of silane ( $\text{SiH}_4$ ) and hydrogen over a heated sapphire or spinel substrate. These deposition constituents (including silicon) react with these substrates and form gaseous reaction products which tend to contaminate the crystalline deposit. At slower growth rates, the increased time of exposure leads to a higher degree of contamination.

Another factor which influences contamination of the grown film is growth temperature. As growth temperatures increase, autodoping with contaminants from the substrate also increases.

Because of the above described difficulties, workers in the art have attempted to minimize the autodoping problem by using as low a growth temperature and as high a growth rate as are consistent with acceptable crystalline perfection and electrical properties in the crystalline deposit.

Active device characteristics tend to be most desirable when the mobility of the charge carriers (Hall mobility) is relatively high, leakage currents are relatively low, and minority carrier lifetime is relatively high. Best MOS/SOS transistor characteristics have been obtained on films  $>0.8 \mu\text{m}$  thick. In general, however, the epitaxial layer thickness should be as thin as possible consistent with acceptable electrical characteristics, since reduced film thickness reduces metallization failure along the film edges where vapor deposited leads are utilized to connect to the electrode regions.

It would be desirable to be able to deposit epitaxial silicon films on sapphire or spinel having a thickness of the order of  $0.5 \mu\text{m}$  which have characteristics for making good electrical devices such as MOS transistors

equal to those made in films one or more  $\mu\text{m}$  thick. In the past, one reason why this has been difficult to achieve, using a growth rate of  $2.0 \mu\text{m}/\text{min}$ , is that only about 15 seconds were available to deposit such a film considering the factors discussed above. This was too short a time to reproducibly manipulate reaction gas flow rates and concentrations so as to alter the conductivity type or carrier concentration at the silicon-substrate interface.

### INVENTION SUMMARY

The present invention is an improved method of depositing an epitaxial film on a crystalline substrate. This is accomplished by depositing a film in two stages by an improved technique. The first stage is the deposition of a very thin film (i.e., one having a thickness of about 500–2000 Å) using a "burst" technique. Using the "burst" technique an average growth rate of 4–6  $\mu\text{m}/\text{min}$  can be achieved. The second stage is the deposition of the remainder of the film at a slower rate (i.e., not over about  $0.5 \mu\text{m}/\text{min}$ ). By this method, a satisfactory silicon film  $0.5 \mu\text{m}$  thick can be deposited in 1–4 minutes.

### THE DRAWING

FIG. 1 is an elevation view, partly in section, of a reaction chamber that can be used in the present method; and

FIG. 2 is a schematic diagram of a gas supply and mixing system which can be used to carry out the method of the present invention.

### DESCRIPTION OF PREFERRED EMBODIMENT

Although the present method can be carried out using either a vertical type or a horizontal type reactor, it will be described in connection with using a barrel type vertical reactor.

Referring to FIG. 1, a suitable reactor may comprise a reaction chamber 2 which is generally bell-shaped. The chamber 2 has inner walls 4 and outer walls 6 so that water may be circulated between the walls to keep the inner walls 4 cool when the chamber is in use.

The top of the chamber 2 is provided with a gas inlet port 8. Suspended from the top of the chamber is a disc-shaped gas deflection means 10. The gas deflection means 10 is disposed near the top of the chamber so as to direct incoming gases toward the walls of the chamber.

The chamber 2 is mounted on a hollow base plate 12 through which cooling water may be circulated by means of an inlet port 14 and an outlet port 16.

Rotatably mounted within the chamber 2 on a vertical spindle 18 is a susceptor 20 which may be made of carbon. The susceptor 20 is shaped like a hexagonal truncated prism, and each of its six sloping faces 22 is provided with a ledge 24 on which a semiconductor wafer 26 may be placed for treatment.

The spindle 18 is mounted on a vertically disposed shaft 28 housed within a sleeve 30 and provided with a bearing 32. The lower end of the shaft 28 is provided with a pulley 34 which is driven through a belt 36 by a variable speed motor 38. In use, the susceptor 20 is slowly rotated as gases are circulated through the chamber 2.

A mixture of reaction gases is delivered to the reaction chamber 2 using the mixing and delivery system 40 as shown in FIG. 2. In the present embodiment, the in-

vention will be described as applied to deposition of an epitaxial silicon film from a doped mixture of silane and hydrogen.

The system 40 includes 3 gas input lines 42, 44 and 46 for delivering a dopant, silane and hydrogen, respectively. The lines 42, 44 and 46 are each provided with gas flow monitoring means 48, 50 and 52, respectively, control valves 54, 56 and 58, respectively, and pressure regulating valves 60, 62 and 64, respectively.

The input lines 42, 44 and 46 are all connected through a control valve 66 to one end of a "burst" chamber 68 which is provided with a pressure gauge 70. In this example, the "burst" chamber is 5 inches long and has a diameter of 2 inches. Connected to the opposite end of the "burst" chamber is an outlet orifice 72 of known diameter. In this example, the diameter of the outlet orifice is 0.050 inch.

Connected into an outlet line 74 from the outlet orifice 72 is a control valve 76. An exhaust line 78 is connected to the outlet line 74 and an exhaust valve 80 controls gas flow through the exhaust line 78.

A branch line 82 connects the outlet from control valve 76 to the gas inlet port 8 of the reaction chamber 2 (FIG. 1).

Another input line 84 connects the single output of 25 a second series of inlet lines (not shown) to the line 84 through a control valve 86.

The above described system may be used to deposit a two-stage composite coating as will now be explained.

First, the "burst" chamber 68 is made ready for the 30 film growth process by flushing it with the gases to be used. Valves 66 and 80 are opened, valve 76 is closed, and valves 54, 56 and 58 are opened to permit flow of dopant gas from the line 42, silane from the line 44 and hydrogen from the line 46, to the "burst" chamber 68. 35 Gas flow-rates are controlled so as to admit a mixture having the proportions 100 cc of dopant gas, which comprises hydrogen, having suspended therein 100 p.p.m. of diborane or arsine (depending upon whether p type or n type doping is desired), 5000 cc of 6% silane in hydrogen and 25,000 cc of hydrogen. These gases are first flushed through the "burst" chamber 68 and the rest of the system including the exhaust line 78 to replace air, and then valve 80 is closed and the burst chamber 68 is filled with the gaseous mixture at 40 60 lbs./sq. in. pressure. When the "burst" chamber 68 is filled, the valve 66 is closed.

The susceptor 20 is then heated to 1000°C by means of rf heating. The susceptor is also rotated at a speed of 18 rpm. The valve 76 is then opened and the gases 50 from the "burst" chamber 68 are suddenly emptied into and through the reaction chamber 2. The gases pass over the heated substrate wafers 26 and begin to deposit an epitaxial layer of silicon thereon. A single crystal layer of silicon approximately 1000 Å thick is 55 deposited in 1 to 1.5 seconds. At the end of this brief period, valve 76 is closed, thus sealing off the "burst" chamber 68 and its associated piping system from the

remainder of the system.

Meanwhile, preparations are also made for growing the remainder of the film at a slower rate by a conventional process. At the same time as the contents of the "burst" chamber 68 are passing through the reaction chamber 2, a mixture having the proportions: 50 cc of hydrogen containing 10 p.p.m. diborane or arsine, 500 cc 6% silane in hydrogen and 25,000 cc of hydrogen are admitted into the reaction chamber 2 by opening the valve 86. This causes an epitaxial film of silicon to continue growing but at a much slower rate.

The second stage of growth can be continued for as long as desired to produce a desired total thickness of silicon. As an example, the slower growth rate may be kept between 0.1 and 0.5 μm/min and the total film thickness may be 0.5 μm.

Both film stages may be doped the same, n type or p type, or one may be doped n type and the other p type. The first stage film may be more highly doped as in this example. In this example, the first stage is doped to about  $10^{17}$  to  $10^{18}$  atoms/cc and the second stage is doped to about  $10^{16}$  atoms/cc.

Although the method has been described in connection with depositing an epitaxial layer of silicon on a sapphire or spinel substrate, it can be used whenever there is danger of unwanted contaminants from the substrate getting into the crystalline layer which is being deposited and thus causing undesirable characteristics to appear in the deposited film.

We claim:

1. A method of comprising a composite layer of heteroepitaxial silicon on a heated sapphire or spinel substrate comprising: depositing a first portion of said layer having a thickness of about 500-2000 Å at an average growth rate of about 4-6 μm/min and the remainder of said layer at a rate of not more than about 0.5 μm/min.
2. A method according to claim 1 in which said first portion of said layer is deposited by pressurizing a gas cylinder with a mixture of silane and hydrogen and allowing the mixture to flow suddenly into the reaction chamber.
3. A method according to claim 2 in which arsine or diborane is included in said mixture.
4. A method according to claim 2 in which said remainder of said layer is deposited immediately following deposition of said first portion of said layer by introducing into said reaction chamber, a mixture of silane and hydrogen having a lower proportion of silane to hydrogen than the mixture in said gas cylinder.
5. A method according to claim 4 in which the mixture in said gas cylinder comprises 5 parts hydrogen to 1 part 6% silane in hydrogen, and the gas mixture for depositing said remainder of said layer comprises 50 parts hydrogen to 1 part 6% silane in hydrogen, all parts being by volume.

\* \* \* \* \*